

## UNITED STATES PATENT OFFICE

2,337,972

## PROCESS OF COATING METALS

William Clayton and Robert Ian Johnson,  
London, and Harry Kenneth Dean, Baildon,  
England, assignors to Crosse & Blackwell  
Limited, London, England, a British company

No Drawing. Application June 27, 1939, Serial  
No. 281,490. In Great Britain June 29, 1938

5 Claims. (Cl. 204—181)

This invention relates to the coating of metal surfaces and to lacquers adapted for such purposes, and more particularly to improved lacquers and methods suitable for protecting the interior of sheet metal containers, such as food containers.

An object of the invention is to provide an improved and inexpensive coating material for metals.

A further object of the invention is to provide a method of applying the coating material so as to obtain a water resistant coating and more particularly a coating which is resistant to attack by water at temperatures at which foodstuffs are normally sterilised.

These and other objects will appear from the following description.

It has been found that drying or semi-drying oils in the raw state and containing a drier can be applied to a clean surface by mechanical means such as rolling, brushing or spraying and, that on stoving (for example for 40 minutes at 350° F.), a film is obtainable which is mechanically hard but which is, nevertheless, unsuitable for coating the interior surface of a sheet metal, for example tinplate, food container since the lacquer is attacked by water at the elevated temperature used in sterilizing the foodstuffs, and is thereby softened.

It has now been found that the requisite water resistance of lacquers, of which the oil components consist of, or contain a large proportion of, raw drying or semi-drying oils, may be achieved if the lacquer is first dispersed in an aqueous medium and then electro-deposited from this dispersion directly on to a metal surface, which functions as anode, in a suitable electric circuit. The resulting deposit, after washing free from adhering drops of the dispersion, drying and stoving, gives a film which is quite suitable for contact with, for example, foodstuffs. The electrodeposited coating for the interior surface of metal containers may be formed at any convenient stage in the fabrication of the said containers. Thus the flat sheets of tinplate from which the containers are to be made, may be coated with the raw oil lacquer by electro-deposition, or the lacquer may be electrically deposited on to the tubular bodies and on to the ends separately. Alternatively raw oil lacquer may be deposited on to the interior, or on to the interior and exterior, of a built up container consisting of the tubular body and one end applied thereto, or having both ends applied where one end is provided with a dispensing orifice through which an electrode may be inserted into the can.

The invention includes the use of those drying oils and semi-drying oils ordinarily used for paints and varnishes, and mixtures of these oils or mixtures of one or more of these oils with a partially oxidised oil, such as a blown oil or a partially polymerised oil, such as stand oil, may be employed. Drying oils such as varnish linseed oil and tung oil, and semi-drying oils, such as pilchard oil, have been found to give satisfactory results.

Various dispersion media may be used but it is preferred to use an aqueous solution of sodium aluminate.

This method of utilising raw oils for coating compositions has been found to have very general application with uniformly excellent results if certain factors are brought under control. For example, where the aqueous system in which the oil is emulsified is such that little or no reinforcing material is co-deposited with the lacquer during the electro-deposition process, for example when the lacquer is emulsified in dilute aqueous solutions of ammonia, then it is desirable, particularly in those cases where the viscosity of the oil phase is naturally low, to increase the viscosity of the oil by the addition of such compounds as aluminium stearate, resins, stand oils, blown oils, etc., as will be found to have the desired effect without impairing the properties of the film. If sodium aluminate solution is used as the aqueous phase then the aluminous compound codeposited with the lacquer is found to bind the film and make it unnecessary to increase the viscosity of the oil.

A proportion of resin may be added when the lacquer is to be deposited upon containers for dry products. This has the advantage that inexpensive resins may be employed so as further to reduce the total costs of the lacquer, which is already less expensive than the lacquers heretofore employed owing to the elimination of the cost of pre-treatment of the oils.

To achieve stoving of lacquer according to the invention, in a period equivalent to the stoving time employed with the usual stoving lacquers, the driers for incorporation in the oils should be selected with care.

*Driers for raw oil lacquers*

Driers may be added to the oils either as insoluble or as soluble salts. Insoluble salts must be heated with oils to high temperatures which are maintained until a clear solution is obtained, this results in a certain amount of darkening, oxidation and polymerisation and cannot be em-

ployed for tung oil. Such "boiled oils" tend to deposit insoluble soaps on standing and must be clarified by storage or filter-pressing. The metal content of the oils is, therefore, somewhat in double unless a quantitative determination is made.

Soluble driers, e. g. naphthenates or linoleates are, therefore, preferably employed since a definite quantity of drier metal can be added either by means of solid salts or their solutions in turpentine or white spirit, and these are the types preferred. A further advantage arising from the use of soluble driers is that less heat treatment is required to effect solution of the drier.

Preferred methods of incorporation are as follows: either (a) the calculated amount of solid linoleate or naphthenate is added to the oil at 150° C. and the temperature raised to 190-200° C., only until a clear solution is obtained, (usually about 5 minutes) and the oil then cooled; or, (b) the calculated quantity of drier is dissolved by heating or intensive stirring in its own weight of turpentine and this solution stirred into the cold oil.

We have found that raw oils need rather different combination of driers from bodied oils and some general features will therefore be outlined.

#### Drying oils

Linseed oil (also perilla, mercuriales, lumbang, i. e. drying oils containing major proportions of linoleic and linolenic acids). Mixtures of cobalt and manganese are suitable for these oils and about 0.05-0.25% of metal having a ratio of cobalt to manganese of between 1:4 and 1:2 or manganese alone may be used but cobalt alone tends to produce rapid surface drying with the result that the film remains a little soft underneath.

Tung oil (also oticica, neou, po-yok, i. e. drying oils whose component acids contain conjugated systems of three double bonds). For these oils we use a drier containing equal amounts of cobalt and manganese, (0.01-0.075%) in conjunction with 0.1-0.3% zinc or lead in order to reduce the frosting of the film. Driers containing zinc or lead should not be heated with the oils but should be added as in method (b). In addition, certain commercial preparations such as Medium 109J (Albert products) can be added to minimise frosting.

#### Semi-drying oils

Soya bean oil (also sunflower, fish, safflower, maize, i. e., semi-drying oils containing major proportions of oleic and linoleic acids). Here the ratio of cobalt to manganese must be increased to between 1:2 and 1:1 and the percentage of metal added may be 0.1 to 0.4%.

The emulsions of these oils are readily prepared by known methods but the best results are obtained when the warm oil (50-100° C.) containing ½-1% added acid (e. g. oleic acid) is run into the agitated alkaline aqueous medium in which case the emulsifying agent (on oleate) will be formed in situ. Emulsions of 30-50% (V/V) disperse phase concentration are generally found most suitable.

The thickness of lacquer films obtained in a given time under specified electrical conditions depends to a large extent on the stability of the emulsion and control is frequently possible by adjustment of the concentration of the emulsifying agent.

The preferred method of carrying out the elec-

trodeposition of these oils is substantially as described in the specifications of co-pending U. S. applications Serial Nos. 88,689 Patent No. 2,215,143 and 94,387 now abandoned or in the specification of co-pending U. S. application Serial No. 189,106 Patent No. 2,215,166, with the difference that it is preferred to use a rather higher initial current density over the surface to be coated than is necessary for other lacquers; for example, when coating tinplate food containers, of which the interior surface area with one end seamed on is 36 sq. inches, the circuit resistance is adjusted to give an initial current of 4-5 amps. with an E. M. F. of 36-40 volts, the stability of the dispersion being adjusted so that a satisfactory film is obtained in 2-4 seconds.

In order to illustrate the invention the following examples are given of emulsions according to the invention suitable for coating metal containers intended for the canning of foodstuffs.

#### Example 1

Into 400 lbs. of varnish linseed oil is incorporated 8 lbs. of cobalt-manganese drier

(Co:Mn=2:8)

by heating to 200° C. When the oil has cooled to 110° C., 4 lbs. of oleic acid is added, and the mixture is emulsified in 60 gallons of softened water containing 1.5% sodium aluminate, at 50° C.

It has been found that varnish linseed oil does not emulsify as readily as, for example, tung oil and the ease with which an emulsion of the linseed oil may be obtained depends to some extent upon the emulsifier used. A high speed propeller unit designed to give a definite circulation under the action of considerable disintegrating forces has been found to give a satisfactory emulsion. The addition of tung oil has also been found to facilitate the emulsification of the linseed oil.

Variations in the type of film obtained on electro-deposition may be secured by (a) varying the concentration of sodium aluminate; (b) varying the amount of oleic acid.

#### Example 2

As in Example 1, but the oil phase consists of a mixture of 90 lbs. of linseed varnish oil and 10 lbs. of linseed stand oil (heavy grade).

#### Example 3

2 lbs. of medium 109J (an anti-frosting agent) dissolved in 2 lbs. toluol, 2 lbs. zinc naphthenate (8% metal) and ½ lb. cobalt naphthenate (6% metal) is stirred into 100 lbs. of cold raw tung oil.

The mixture is heated to 60° C. and emulsified as in Example 1, oleic acid being added to the oil if necessary.

#### Example 4

88 lbs. of pilchard oil and 12 lbs. raw tung oil is heated to 200° C., 4 lbs. of cobalt manganese drier (10% metal concentration) (Co:Mn=1:2) being added when the temperature reaches 150° C.

The oil is then cooled to 110° C., ½ lb. of oleic acid is added and the mixture emulsified as in Example 1.

The full importance of the invention lies not only in the excellence of the films produced by this method but further in the considerable economic and technical advantages resulting from the use of these coating compositions. For ex-

ample, no expensive oil blowing or polymerizing plant is required as in most cases, the raw oil as supplied can (after incorporation of the suitable driers) be immediately emulsified in the appropriate aqueous system and used for electro-deposition. The conventional lacquer manufacturing plant, with its time consuming processes, is completely eliminated. Furthermore the water repellent character of these raw oil lacquer films makes the stage of washing the deposited film very much easier than in the case of films of deposited lacquers of other types.

The electrodeposition of raw oil lacquers may follow known pre-treatments of the metal surface which are designed to improve the resistance to discolouration by sulphur compounds in the pack, or to improve the adhesion of the lacquer. For example, the surface of the tinplate to be coated may be subjected to anodic oxidation, for example in the manner described in the specification of copending U. S. application Serial No. 145,691 Patent No. 2,215,165, or a metallic oxide, such as aluminium oxide, may be deposited upon the surface by making the surface an electrode in a suitable electrolytic bath and the lacquer may then be applied to the pre-treated surface as described above.

Instead of anodically pre-treating the tinplate surface this may be oxidised or provided with a metallic oxide coating by purely chemical treatment, for example the tinplate may be immersed in a suitable oxidising solution or it may be heated in an oxidising atmosphere so as to provide the oxide coating.

The lacquer and the processes according to the invention are applicable to the coating of any metallic surface, for example tinplate, black plate or aluminium.

Having thus described the invention, what we claim as new and desire to secure by Letters Patent is:

1. The process of forming a protective coating on a metal surface, said coating being capable of resisting attack by water at the temperature at which foodstuffs are normally sterilised, which comprises preparing a dispersion of a raw drying oil and an oil-soluble drier in an aqueous alkaline dispersion medium, electrolytically provoking a deposit from the dispersion upon the metal surface as anode to provide an adherent film containing the oil and drier with the oil constituting the preponderant coating component, and then washing, drying and stoving the deposited coating film.

2. The process of forming a protective coating on a metal surface, said coating being capable of resisting attack by water at the temperature at which foodstuffs are normally sterilised, which comprises preparing a dispersion of a raw drying oil and an oil-soluble drier in an ammoniacal aqueous alkaline dispersion medium, electrolytically provoking a deposit from the dispersion upon the metal surface as anode to provide an adherent film containing the oil and drier with the oil constituting the preponderant coating component, and then washing, drying and stoving the deposited coating film.

3. The process of forming a protective coating on a metal surface, said coating being capable of resisting attack by water at the temperature at which foodstuffs are normally sterilised, which

5 comprises preparing a dispersion of a raw drying oil and a drier in an aqueous alkaline sodium aluminate solution in the presence of a quantity of oleic acid corresponding to substantially one-half to one per cent of the amount of oil, the drier being an oil-soluble mixture of cobalt and manganese salts having a metal concentration of 0.01 to 0.4 per cent based on the oil and with a cobalt:manganese ratio of essentially 1:4 to 1:1, electrolytically provoking a deposit from the dispersion upon the metal surface with said surface as anode and at a current density of substantially 4 to 5 amperes per 36 square inches to provide a film containing the oil and drier with the oil constituting the preponderant coating component, and then washing, drying and stoving the deposited coating film.

4. The process of forming a protective coating on a metal surface, said coating being capable of resisting attack by water at the temperature at

25 which foodstuffs are normally sterilised, which comprises preparing a dispersion of a raw drying oil whose component acids contain conjugated systems of three double bonds in the molecule, together with an oil-soluble drier, in an aqueous alkaline sodium aluminate solution, the drier being an oil-soluble mixture of equal amounts of cobalt and manganese salts having a metal concentration of 0.01 to 0.075 per cent of each based on the oil, electrolytically provoking a deposit from the dispersion upon the metal surface with said surface as anode and at a current density of substantially 4 to 5 amperes per 36 square inches to provide a film containing the oil and drier with the oil constituting the preponderant coating component, and then washing, drying and stoving the deposited coating film.

5. The process of forming a protective coating on a metal surface, said coating being capable of resisting attack by water at the temperature at

45 which foodstuffs are normally sterilised, which comprises preparing a dispersion of a raw drying oil of the kind having linoleic and linolenic acids as the major acid component in the oil molecules, together with a drier, in an aqueous alkaline sodium aluminate solution, the drier being an oil-soluble mixture of cobalt and manganese salts having a metal concentration of 0.01 to 0.25 per cent based on the oil and with a cobalt:manganese ratio of essentially 1:4 to 1:2, electrolytically provoking a deposit from the dispersion upon the metal surface with said surface as anode and at a current density of substantially 4 to 5 amperes per 36 square inches to provide a film containing the oil and drier with the oil constituting the preponderant coating component, and then washing, drying and stoving the deposited coating film.

55

60

65

HARRY KENNETH DEAN.  
WILLIAM CLAYTON.  
ROBERT IAN JOHNSON.